# EUROPEAN PATENT SPECIFICATION

(11) **EP 1 460 650 B1**
(45) Date of publication and mention of the grant of the patent: **14.11.2007**
(21) Application number: 03748612.3
(22) Date of filing: 30.09.2003
(51) Int. Cl.: C22C 1/04, C22C 33/02, H01F 1/057, H01F 1/053, H01F 1/047

(54) **R-T-B BASED RARE EARTH ELEMENT PERMANENT MAGNET**
SELTENERDELEMENT-PERMANENTMAGNET AUF R-T-B-BASIS
AIMANT PERMANENT A ELEMENTS EN TERRES RARES EN ALLIAGE DE R-T-B

(30) Priority: 30.09.2002 JP 2002287033; 28.03.2003 JP 2003092890
(43) Date of publication of application: 22.09.2004
(73) Proprietor: TDK Corporation, Chuo-ku, Tokyo 103-8272 (JP)
(72) Inventor: Ishizaka, Chikara, Tokyo 103-8272 (JP); Nishizawa, Gouichi, Tokyo 103-8272 (JP); Hidaka, Tetsuya, Tokyo 103-8272 (JP); Fukuno, Akira, Tokyo 103-8272 (JP); Uchida, Nobuya, Tokyo 103-8272 (JP)
(74) Representative: HOFFMANN EITLE
(86) International application number: PCT/JP2003/012491
(87) International publication number: WO 2004/029999

(56) References cited:
- EP-A- 0 242 187
- EP-A- 0 302 395
- EP-A- 1 014 392
- EP-A- 1 164 599
- WO-A1-00/12771
- JP-A- 1 196 104
- JP-A- 7 130 522
- JP-A- 7 176 414
- JP-A- 9 223 617
- JP-A- 10 064 712
- JP-A- 2002 075 717
- JP-A- 2002 093 610
- JP-A- 2002 164 239
- US-A- 4 895 607
- KIM A S ET AL: "MICROSTRUCTURE OF ZR CONTAINING NDFEB" IEEE TRANSACTIONS ON MAGNETICS, IEEE INC. NEW YORK, US, vol. 33, no. 5, PART 2, September 1997 (1997-09), pages 3823-3825, XP000703229 ISSN: 0018-9464
- POLLARD R J ET AL: "EFFECT OF ZR ADDITIONS ON THE MICROSTRUCTURAL AND MAGNETIC PROPERTIES OF NDFEB BASED MAGNETS" IEEE TRANSACTIONS ON MAGNETICS, IEEE INC. NEW YORK, US, vol. 24, no. 2, 1 March 1988 (1988-03-01), pages 1626-1628, XP000174162 ISSN: 0018-9464
- BESENICAR S: "THE INFLUENCE OF ZRO2 ADDITION ON THE MICROSTRUCTURE AND THE MAGNETIC PROPERTIES OF ND-DY-FE-B MAGNETS" JOURNAL OF MAGNETISM AND MAGNETIC MATERIALS, ELSEVIER SCIENCE PUBLISHERS, AMSTERDAM, NL, vol. 104 - 107, no. PART 2, 1 February 1992 (1992-02-01), pages 1175-1178, XP000329968 ISSN: 0304-8853
- PATENT ABSTRACTS OF JAPAN vol. 1998, no. 14, 31 December 1998 (1998-12-31) -& JP 10 259459 A (MITSUBISHI MATERIALS CORP), 29 September 1998 (1998-09-29)
- PATENT ABSTRACTS OF JAPAN vol. 1998, no. 06, 30 April 1998 (1998-04-30) -& JP 10 041113 A (MITSUBISHI MATERIALS CORP), 13 February 1998 (1998-02-13)

## Description

### TECHNICAL FIELD

The present invention relates to an R-T-B system rare earth permanent magnet containing, as main components, R (wherein R represents one or more rare earth elements, providing that the rare earth elements include Y), T (wherein T represents at least one transition metal element essentially containing Fe, or Fe and Co), and B (boron).

### BACKGROUND ART

Among rare earth permanent magnets, an R-T-B system rare earth permanent magnet has been increasingly demanded year by year for the reasons that its magnetic properties are excellent and that its main component Nd is abundant as a source and relatively inexpensive.

Research and development directed towards the improvement of the magnetic properties of the R-T-B system rare earth permanent magnet have intensively progressed. For example, Japanese Patent Laid-Open No. 1-219143 discloses that the addition of 0.02 to 0.5 at % of Cu improves magnetic properties of the R-T-B system rare earth permanent magnet as well as heat treatment conditions. However, the method described in Japanese Patent Laid-Open No. 1-219143 is insufficient to obtain high magnetic properties required of a high performance magnet, such as a high coercive force (HcJ) and a high residual magnetic flux density (Br).

The magnetic properties of an R-T-B system rare earth permanent magnet obtained by sintering depend on the sintering temperature. On the other hand, it is difficult to equalize the heating temperature throughout all parts of a sintering furnace in the scale of industrial manufacturing. Thus, the R-T-B system rare earth permanent magnet is required to obtain desired magnetic properties even when the sintering temperature is changed. A temperature range in which desired magnetic properties can be obtained is referred to as a suitable sintering temperature range herein.

In order to obtain a higher-performance R-T-B system rare earth permanent magnet, it is necessary to decrease the amount of oxygen contained in alloys. However, if the amount of oxygen contained in the alloys is decreased, abnormal grain growth is likely to occure in a sintering process, resulting in a decrease in a squareness. This is because oxides formed by oxygen contained in the alloys inhibit the grain growth.

Thus, a method of adding a new element to the R-T-B system rare earth permanent magnet containing Cu has been studied as means for improving the magnetic properties. Japanese Patent Laid-Open No. 2000-234151 discloses the addition of Zr and/or Cr to obtain a high coercive force and a high residual magnetic flux density.

Likewise, Japanese Patent Laid-Open No. 2002-75717 discloses a method of uniformly dispersing a fine ZrB compound, NbB compound or HfB compound (hereinafter referred to as an M-B compound) into an R-T-B system rare earth permanent magnet containing Zr, Nb or Hf as well as Co, Al and Cu, followed by precipitation, so as to inhibit the grain growth in a sintering process and to improve magnetic properties and the suitable sintering temperature range.

According to Japanese Patent Laid-Open No. 2002-75717, the suitable sintering temperature range is extended by the dispersion and precipitation of the M-B compound. However, in Example 3-1 described in the above publication, the suitable sintering temperature range is narrow, such as approximately 20°C. Accordingly, to obtain high magnetic properties using a mass-production furnace or the like, it is desired to further extend the suitable sintering temperature range. Moreover, in order to obtain a sufficiently wide suitable sintering temperature range, it is effective to increase the additive amount of Zr. However, as the additive amount of Zr increases, the residual magnetic flux density decreases, and thus, high magnetic properties of interest cannot be obtained

Kim A S et al (IEEE Trains. On Magnetics, US, vol.33, no.5, part 2, p.3823/5) discusses the microstructure of Zr containing Nd (Dy) FeB alloys. The effect of various Zr contents on the coercivity was studied to determine the optimum Zr level.

Pollard R J et al (IEEE Trans. On Magnetics, US, vol.24, no.2, p.1626/8) relates to the effect of Zr additions on the micro structural and magnetic properties of NdFeB based magnets.

Benesicar et al (Journal of magnetism and magnetic materials, Elsevier Sc.Publ., NL, vol. 104-107, part 2, p. 1175/8) discusses the influence of ZrO₂ addition on the microstructure and the magnetic properties of NdDyFeB magnets.

Hence, it is an object of the present invention to provide an R-T-B system rare earth permanent magnet, which enables to inhibit the grain growth, while keeping a decrease in magnetic properties to a minimum, and also enables to further improve the suitable sintering temperature range.

### DISCLOSURE OF THE INVENTION

The present inventor has found that when a product that is rich in Zr exists in an R₂T₁₄B phase constituting the main phase of an R-T-B system rare earth permanent magnet, the permanent magnet enables to inhibit the grain growth, while keeping a decrease in magnetic properties to a minimum, and to improve the suitable sintering temperature range. That is to say, the present invention provides an R-T-B system rare earth permanent magnet, which is a sintered body consisting of 28% to 33% by weight of R, 0.5% to 1.5% by weight of B, 0.03% to 0.3% by weight of Al, 0.03% to 0.3% by weight of Cu, 0.05% to 0.2% by weight or Zr, 0.1% to 4% by weight of Co, and the balance being Fe and unavoidable impurities; said sintered body comprising a main phase consisting of an R₂T₁₄B phase, wherein R represents one or more rare earth elements providing that the rare earth elements include Y, and T represents one or more transition metal elements containing Fe, or Fe and Co, and a grain boundary phase containing a higher amount of R than the above main phase, wherein a product that is rich in Zr exists in the above R₂T₁₄B phase and has a length of several hundreds nm and a width between several nm and 15 nm.

In the R-T-B system rare earth permanent magnet of the present invention, the product that is rich in Zr has a platy or acicular form.

In the R-T-B system rare earth permanent magnet of the present invention, the amount of oxygen contained in the above sintered body is preferably 2, 000 ppm or less. This is because effects obtained by the presence of the Zr rich product in the R₂T₁₄B phase, such as the inhibition of the grain growth or the extension of the suitable sintering temperature range become significant, when the amount of oxygen contained in the sintered body is as low as 2,000 ppm or less.

In the R-T-B system rare earth permanent magnet of the present invention, the sintered body preferably has a composition consisting of 28% to 33% by weight of R, 0.5% to 1.5% by weight of B, 0.03% to 0.3% by weight of Al, 0.03% to 0.3% by weight of Cu, 0.05% to 0.2% by weight of Zr, 0.1% to 4% by weight of Co, and the balance substantially being Fe.

In the R-T-B system rare earth permanent magnet of the present invention, Zr is contained in the sintered body, more preferably within the range between 0. 1% and 0.15% by weight.

### BRIEF DESCRIPTION OF THE DRAWINGS

FIG. 1 is a table showing the combinations of low R alloys and high R alloys used in Embodiment Example 1, and the compositions of the obtained permanent magnets;
FIG. 2 is a table showing the magnetic properties of the permanent magnets obtained in Embodiment Example 1;
FIG. 3 is a graph showing the relationship between the amount of additive element M (Zr or Ti) and the residual magnetic flux density (Br) of each of the permanent magnets obtained in Embodiment Example 1;
FIG. 4 is a graph showing the relationship between the amount of additive element M (Zr or Ti) and the coercive force (HcJ) of each of the permanent magnets obtained in Embodiment Example 1;
FIG. 5 is a graph showing the relationship between the amount of additive element M (Zr or Ti) and the squareness (Hk/HcJ) of each of the permanent magnets obtained in Embodiment Example 1;
FIG. 6 is a TEM (Transmission Electron Microscope) photograph of a sample (containing 0.10% by weight of Zr) of Example 1;
FIG. 7A is a diagram showing an EDS (Energy Dispersive X-ray Fluorescence Spectrometer) profile of a product existing in the sample (containing 0.10% by weight of Zr) of Example 1;
FIG. 7B is a diagram showing an EDS profile of the R₂T₁₄B phase of the sample (containing 0.10% by weight of Zr) of Example 1;
FIG. 8 is a high resolution TEM photograph of the sample (containing 0.10% by weight of Zr) of Example 1;
FIG. 9 is a TEM photograph of the sample (containing 0.10% by weight of Zr) of Example 1;
FIG. 10 is another TEM photograph of the sample (containing 0.10% by weight of Zr) of Example 1;
FIG. 11A is a photograph (lower) showing the Zr mapping results of the sample (containing 0.10% by weight of Zr) of Example 1 by EPMA (Electron Probe Micro Analyzer), and a photograph (upper) showing a composition image in the same scope as the Zr mapping results (lower);
FIG. 11B is a photograph (lower) showing the Zr mapping results of a sample (containing 0.10% by weight of Zr) of Comparative Example 2 by EPMA, and a photograph (upper) showing a composition image in the same scope as the Zr mapping results (lower);
FIG. 12 is a table showing the magnetic properties of the permanent magnets obtained in Embodiment Example 2;
FIG. 13 is a graph showing the relationship between the sintering temperature and the residual magnetic flux density (Br) in Embodiment Example 2;
FIG. 14 is a graph showing the relationship between the sintering temperature and the coercive force (HcJ) in Embodiment Example 2;
FIG. 15 is a graph showing the relationship between the sintering temperature and the squareness (Hk/HcJ) in Embodiment Example 2;
FIG. 16 is a graph showing the correspondence between the residual magnetic flux density (Br) and the squareness (Hk/HcJ) at each sintering temperature in Embodiment Example 2;
FIG. 17 is a table showing the combinations of low R alloys and high R alloys used in Embodiment Example 3, and the compositions of the obtained permanent magnets;
FIG. 18 is a table showing the magnetic properties of the permanent magnets obtained in Embodiment Example 3;
FIG. 19 is a table showing the combinations of low R alloys and high R alloys used in Embodiment Example 4, and the compositions of the obtained permanent magnets;
FIG. 20 is a table showing the magnetic properties of the permanent magnets obtained in Embodiment Example 4.

### BEST MODE FOR CARRYING OUT THE INVENTION

The embodiments of the present invention will be described below.

### <Microstructure>

The R-T-B system rare earth permanent magnet of the present invention comprises a sintered body consisting essentially of 28% to 33% by weight of R, 0.5% to 1.5% by weight of B, 0.03% to 0.3% by weight of Al, 0.08% to 0.3% by weight of Cu, 0.05% to 0.2% by weight or Zr, 0.1% to 4% by weight of Co, and the balance being Fe and unavoidable impurities, said sintered body comprising a main phase consisting of a R₂T₁₄B phase (wherein R represents one or more rare earth elements (providing that the rare earth elements include Y), and T represents one or more transition metal elements containing Fe, or Fe and Co), and a grain boundary phase containing a higher amount of R than the main phase. The present invention is characterized in that a product that is rich in Zr, and which has a length of several hundreds nm and a width between several nm and 15 nm, exists in the R₂T₁₄B phase.

The R-T-B system rare earth permanent magnet containing this product enables to inhibit the grain growth, while keeping a decrease in magnetic properties to a minimum, and to extend the suitable sintering temperature range. This product needs to exist in the R₂T₁₄B phase, but it is not required to exist in all the R₂T₁₄B phases. This product may exist also in the grain boundary phase. However, when the Zr rich product exists only in the grain boundary phase, the effects of the present invention cannot be obtained.

In the R-T-B system rare earth permanent magnet, Ti has conventionally been known as an additive element that forms the product in the R₂T₁₄B phase (e.g., J. Appl. Phys. 69 (1991) 6055). The present inventors have found that the formation of the product in the R₂T₁₄B phase by addition of Zr or Ti is effective for the extension of a suitable sintering temperature range. In the case of adding Zr, although Zr is added in an amount necessary to obtain such an effect as the extension of a suitable sintering temperature range, it causes almost no decrease in magnetic properties, and more specifically, almost no decrease in the residual magnetic flux density (Br). On the other hand, in the case of adding Ti, if this element is added in an amount necessary to obtain such an effect as the extension of a suitable sintering temperature range, the residualmagnetic flux density (Br) is significantlydecreased, and thus, it is clear that the addition of Ti is not practically preferable. As stated above, when the composition of the product is rich in Zr, it makes possible to consistently produce permanent magnets with high magnetic properties in a wide suitable sintering temperature range.

The present inventors have confirmed that in order to allow the product that is rich in Zr to exist in the R₂T₁₄B phase, there are several requirements on the manufacturing method. The procedure of the manufacturing method of the permanent magnet of the present invention will be described later. The requirements to allow the Zr rich product to exist in the R₂T₁₄B phase will be explained below.

There are two methods for manufacturing an R-T-B system rare earth permanent magnet: a method of using as a starting alloy a single alloy having a desired composition (hereinafter referred to as a single method), andamethodof using as starting alloys a plurality of alloys having different compositions (hereinafter referred to as a mixing method). In the mixing method, alloys containing an R₂T₁₄B phase as a main constituent (low R alloys) and alloys containing a higher amount of R than the low R alloys (high R alloys) are typically used, as starting alloys.

The present inventors added Zr to either the low R alloys or the high R alloys, so as to obtain an R-T-B system rare earth permanent magnet. As a result, the present inventors confirmed that when Zr is added to the low R alloys in order to produce a permanent magnet, the product that is rich in Zr exists in the R₂T₁₄B phase. The present inventors also confirmed that when Zr is added to the high R alloys, the Zr rich product does not exist in the R₂T₁₄B phase.

Moreover, even in the case where Zr is added to the low R alloys, if the Zr rich product existed in the R₂T₁₄B phase in the low R alloy stage, it was not confirmed that the Zr rich product exists in the R₂T₁₄B phase after a sintering process, although it existed in an R rich phase (grain boundary phase) located at a triple point in the microstructure of the sintered bodies. Accordingly, in order to allow the Zr rich product to exist in the R₂T₁₄B phase of the R-T-B system rare earth permanent magnet, it is important not to allow the Zr rich product to exist in the R₂T₁₄B phase in the mother alloy stage.

On that account, a method for manufacturing mother alloys should be considered. When the low R alloys are manufactured by the strip casting method, the peripheral velocity of a chill roll needs to be controlled. When the peripheral velocity of a chill roll is low, it results in the deposition of α-Fe, and the Zr rich product is generated in the R₂T₁₄B phase of the low R alloys. As a result of studies of the present inventors, it was found that when the peripheral velocity of a chill roll is within the range between 1.0 and 1.8 m/s, low R alloys in which the Zr rich product do not exist in the R₂T₁₄B phase can be obtained. Using the obtained low R alloys, a permanent magnet with high magnetic properties can be obtained.

Furthermore, even in the case of obtaining low R alloys in which the Zr rich product does not exist in the R₂T₁₄B phase, it is not desired in the present invention that the obtained low R alloys are subjected to a heat treatment and then used as mother alloys. This is because the Zr rich product is generated in the R₂T₁₄B phase of the low R alloys as a result of undergoing a heat treatment in a temperature area (approximately 700°C or higher) where the microstructure of the low R alloys may be modified.

### <Chemical composition>

Next, a desired composition of the R-T-B system rare earth permanent magnet of the present invention will be explained. The term chemical composition is used herein to mean a chemical composition obtained after sintering.

The rare earth permanent magnet of the present invention contains 28% to 33% by weight of R.

The term R is used herein to mean one or more rare earth elements selected from a group consisting of La, Ce, Pr, Nd, Sm, Eu, Gd, Tb, Dy, Ho, Er, Yb, Lu and Y. If the amount of R is less than 28% by weight, an R₂T₁₄B₁ phase as a main phase of the rare earth permanent magnet is not sufficiently generated. Accordingly, α-Fe or the like having soft magnetism is deposited and the coercive force significantly decreases. On the other hand, if the amount of R exceeds 35% by weight, the volume ratio of the R₂T₁₄B phase as a main phase decreases, and the residual magnetic flux density decreases. Moreover, if the amount of R exceeds 33% by weight, R reacts with oxygen, and the content of oxygen thereby increases. In accordance with the increase of the oxygen content, an R rich phase effective for the generation of coercive force decreases, resulting in a reduction in the coercive force. Therefore, the amount of R is set between 28% and 33% by weight. The amount of R is preferably between 29% and 32% by weight.

SinceNd is abundant as a source and relatively inexpensive, it is preferable to use Nd as a main component of R. Moreover, since the containment of Dy increases an anisotropic magnetic field, it is effective to contain Dy to improve the coercive force. Accordingly, it is desired to select Nd and Dy for R and to set the total amount of Nd and Dy between 28% and 33% by weight. In addition, in the above range, the amount of Dy is preferably between 0.1% and 8% by weight. It is desired that the amount of Dy is arbitrarily determined within the above range, depending on which is more important, a residual magnetic flux density or a coercive force. This is to say, when a high residual magnetic flux density is required to be obtained, the amount of Dy is preferably set between 0.1% and 3.5% by weight. When a high coercive force is required to be obtained, it is preferably set between 3.5% and 8% by weight.

Moreover, the rare earth permanent magnet of the present invention contains 0.5% to 1.5 % by weight of boron (B). If the amount of B is less than 0.5% by weight, a high coercive force cannot be obtained. However, if the amount of B exceeds 1.5% by weight, the residual magnetic flux density is likely to decrease. Accordingly, the upper limit is set at 1.5% by weight. The amount of B is preferably between 0.8% and 1.2% by weight.

The R-T-B system rare earth permanent magnet of the present invention may contain Al and Cu within the range between 0.03% and 0.3% by weight. The containment of Al and Cu within the above range can impart a high coercive force, a strong corrosion resistance, and an improved temperature stability of magnetic properties to the obtained permanent magnet. The additive amount of Al is preferably between 0.05% and 0.25% by weight. The additive amount of Cu is preferably between 0.03% and 0.15%, and more preferably between 0.03% and 0.08% by weight.

In order to allow the Zr rich product to exist in the R₂T₁₄B phase, the R-T-B system rare earth permanent magnet of the present invention contains Zr within the range between 0.05% and 0.2% by weight. When the content of oxygen is reduced to improve the magnetic properties of the R-T-B system rare earth permanent magnet, Zr exerts the effect of inhibiting the abnormal grain growth in a sintering process and thereby makes the microstructure of the sintered body uniform and fine. Accordingly, when the amount of oxygen is low, Zr fully exerts its effect. The amount of Zr is preferably between 0.1% and 0.15% by weight.

The R-T-B system rare earth permanent magnet of the present invention contains 2,000 ppm or less oxygen. If it contains a large amount of oxygen, an oxide phase that is a non-magnetic component increases, thereby decreasing magnetic properties. Thus, in the present invention, the amount of oxygen contained in a sintered body is set at 2,000 ppm or less, preferably 1,500 ppm or less, and more preferably 1,000 ppm or less. However, when the amount of oxygen is simply decreased, an oxide phase having a grain growth inhibiting effect decreases, so that the grain growth easily occures in a process of obtaining full density increase during sintering. Thus, in the present invention, the R-T-B system rare earth permanent magnet to contains a certain amount of Zr, which exerts the effect of inhibiting the abnormal grain growth in a sintering process.

The R-T-B system rare earth permanent magnet of the present invention contains Co in an amount of 0.1% and 4% by weight, preferably between 0.1% and 2.0% by weight, and more preferably between 0.3% and 1.0% by weight. Co forms a phase similar to that of Fe. Co has an effect to improve Curie temperature and the corrosion resistance of a grain boundary phase.

### <Manufacturing method>

Next, the suitable method for manufacturing an R-T-B system rare earth permanent magnet of the present invention will be explained.

Embodiments of the present invention show a method for manufacturing a rare earth permanent magnet using alloys (low R alloys) containing an R₂T₁₄B phase as a main phase and other alloys (high R alloys) containing a higher amount of R than the low R alloys.

Raw material is first subjected to strip casting in a vacuum or an inert gas atmosphere, or preferably an Ar atmosphere, so that low R alloys and high R alloys are obtained. As stated above, it is necessary to give special consideration to the obtained strips, especially to the strips of the low R alloys, so that a Zr rich product is not generated in the R₂T₁₄B phase. More specifically, the peripheral velocity of a chill roll is set within the range between 1.0 and 1.8 m/s. The preferred peripheral velocity of a chill roll is between 1.2 and 1.5 m/s.

It is important for the present invention not to allow a Zr rich product to generate in an R₂T₁₄B phase during the period from the achievement of low R alloys having the R₂T₁₄B phase in which the present Zr rich product does not exist until a sintering process described later. In other words, it is important for the present invention to maintain the form of the above R₂T₁₄B phase. For example, it is preferable not to carry out a heat treatment, in which the low R alloys are heated to 700°C or higher and retained, before crushing processes that begin with hydrogen crushing. This point will be further described in Embodiment Example 1 described later.

The feature of the present embodiment is that Zr is added to low R alloys. As explained above in the column <Microstructure>, the reason is that the Zr rich product can be allowed to exist in the R₂T₁₄B phase of the R-T-B system rare earth permanent magnet by adding Zr to low R alloys containing no Zr rich products in an R₂T₁₄B phase thereof. The low R alloys can contain Cu and Al, in addition to rare earth elements, Fe, Co and B. Moreover, the high R alloys can also contain Cu and Al, in addition to rare earth element, Fe, Co and B.

After preparing the low R alloys and the high R alloys, these master alloys are crushed separately or together. The crushing step comprises a crushing process and a pulverizing process. First, each of the master alloys is crushed to a particle size of approximately several hundreds of µm. The crushing is preferably carried out in an inert gas atmosphere, using a stamp mill, a jaw crusher, a brown mill, etc. In order to improve rough crushability, it is effective to carry out crushing after the absorption of hydrogen. Otherwise, it is also possible to release hydrogen after absorbing it and then carry out crushing.

After carrying out the crushing, the routine proceeds to a pulverizing process. In the pulverizing process, a jet mill is mainly used, and crushed powders with a particle size of approximately several hundreds of µm are pulverized to a mean particle size between 3 and 5 µm. The jet mill is a method comprising releasing a high-pressure inert gas (e.g., nitrogen gas) from a narrow nozzle so as to generate a high-speed gas flow, accelerating the crushed powders with the high-speed gas flow, and making crushed powders hit against each other, the target, or the wall of the container, so as to pulverize the powders.

When the low R alloys and the high R alloys are pulverized separately in the pulverizing process, the pulverized low R alloy powders are mixed with the pulverized high R alloy powders in a nitrogen atmosphere. The mixing ratio of the low R alloy powders and the high R alloy powders may be approximately between 80 : 20 and 97 : 3 at a weight ratio. Likely, in a case where the low R alloys are pulverized together with the high R alloys, the mixing ratio may be approximately between 80 : 20 and 97 : 3 at a weight ratio. When approximately 0.01% to 0.3% by weight of additive agents such as zinc stearate is added during the pulverizing process, fine powders which are well oriented, can be obtained during compacting.

Subsequently, mixed powders comprising of the low R alloy powders and the high R alloy powders are filled in a tooling equipped with electromagnets, and they are compacted in a magnet field, in a state where their crystallographic axis is oriented by applying a magnetic field. This compacting may be carried out by applying a pressure of approximately 0.7 to 1.5 t/cm² in a magnetic field of 12.0 to 17.0 kOe.

After the mixed powders are compacted in the magnetic field, the compacted body is sintered in a vacuum or an inert gas atmosphere. The sintering temperature needs to be adjusted depending on various conditions such as a composition, a crushing method, the difference between particle size and particle size distribution, but the sintering may be carried out at 1, 000°C to 1,100°C for about 1 to 5 hours. In the present invention, the Zr rich product is generated in the R₂T₁₄B phase in this sintering process. The mechanism of generating after sintering the Zr rich product that did not exist in the low R alloy stage is unknown, but there is a possibility that Zr dissolved in the R₂T₁₄B phase in the low R alloy stage might be deposited therein during the sintering process.

After completion of the sintering, the obtained sintered body may be subjected to an aging treatment. The aging treatment is important for the control of a coercive force. When the aging treatment is carried out in two steps, it is effective to retain the sintered body for a certain time at around 800°C and around 600°C. When a heat treatment is carried out at around 800°C after completion of the sintering, the coercive force increases. Accordingly, it is particularly effective in the mixing method. Moreover, when a heat treatment is carried out at around 600°C, the coercive force significantly increases. Accordingly, when the aging treatment is carried out in a single step, it is appropriate to carry out it at around 600°C.

### (EMBODIMENT EXAMPLES)

### <Embodiment Example 1>

An R-T-B system rare earth permanent magnet was manufactured by the following manufacturing process.

### (1) Mother alloys

Mother alloys (strips) having compositions and thicknesses shown in FIG. 1 were prepared by the strip casting method. The roll peripheral velocity of low R alloys was set to 1.5 m/s, and that of high R alloys was set to 0. 6m/s. However, the roll peripheral velocity of the low R alloys in Comparative Example 3 shown in FIG. 1 was set to 0.6 m/s. The thickness of alloys was a mean value obtained by measuring the thicknesses of 50 strips. It was confirmed that a Zr rich product (hereinafter referred to as an intraphase product) was not observed in the R₂T₁₄B phase of the low R alloys of Example 1 as shown in FIG. 1, but that the intraphase product existed in the R₂T₁₄B phase of the low R alloys of Comparative Example 3 as shown in the same figure.

### (2) Hydrogen crushing process

A hydrogen crushing treatment was carried out, in which after hydrogen was absorbed at room temperature, dehydrogenation was carried out thereon at 600°C for 1 hour in an Ar atmosphere.

To control the amount of oxygen contained in a sintered body to 2,000 ppm or less, so as to obtain high magnetic properties, in the present experiments, the atmosphere was controlled at an oxygen concentration less than 100 ppm throughout processes, from a hydrogen treatment (recovery after a crushing process) to sintering (input into a sintering furnace).

### (3) Mixing and crushing processes

Generally, two-step crushing is carried out, which includes crushing process and pulverizing process. However, the crushing process was omitted in the present Examples.

Before carrying out the pulverizing process, 0.05% by weight of zinc stearate was added. Thereafter, using a Nauta Mixer, the low R alloys were mixed with the high R alloys for 30 minutes in the combination of each of Example 1 and Comparative Examples 1 to 3 as shown in FIG. 1. In all of Example 1 and Comparative Examples 1 to 3, the mixing ratio between the low R alloys and the high R alloys was 90 : 10.

Thereafter, the mixture was subjected to the pulverizing with a jet mill to a mean particle size of 4.8 to 5.1 µm.

### (4) Compacting process

The obtained fine powders were compacted in a magnetic field of 15.0 kOe by applying a pressure of 1.2 t/cm², so as to obtain a compacted body.

### (5) Sintering and aging processes

The obtained compacted body was sintered at 1, 070°C for 4 hours in a vacuum atmosphere, followed by quenching. Thereafter, the obtained sintered body was subjected to a two-step aging treatment consisting of treatments of 800°C × 1 hour and 550°C × 2.5 hours (both in an Ar atmosphere).

The magnetic properties of the obtained permanent magnets were measured with a B-H tracer. The results are shown in FIGS. 2 to 5. In FIGS. 2 to 5, Br represents a residual magnetic flux density, HcJ represents a coercive force, and "Hk/HcJ" means a squareness. The squareness (Hk/HcJ) is an index of magnetic performance, and it represents an angular degree in the second quadrant of a magnetic hysteresis loop. Furthermore, Hk means an external magnetic field strength obtained when the magnetic flux density becomes 90% of the residual magnetic flux density in the second quadrant of a magnetic hysteresis loop. In FIGS. 2 to 5, a permanent magnet in which an intraphase product was observed is marked with a circle (○), and a permanent magnet in which the product was not observed is marked with a cross(×). The presence or absence of an intraphase product was confirmed based on observation with TEM (Transmission Electron Microscope, JEM-3010 manufactured by Japan Electron Optics Laboratory Co., Ltd). The sample for the observation was obtained by the ion-milling method, and the C plane of the R₂T₁₄B phase was observed. It is noted that the chemical compositions of the obtained sintered body are shown in the column "Composition of sintered body" in FIG. 1. Further, no intraphase products were observed in Comparative Example 3, but the Zr rich product was observed in a grain boundary phase thereof.

From FIGS. 2 and 5, it is found that in R-T-B system rare earth permanent magnets in which an intraphase product was observed (Example 1 and Comparative Example 1), the abnormal grain growth was inhibited and the squareness (Hk/HcJ) was improved by adding only a small amount of additive element M (Zr or Ti). However, in a case where Ti was selected as an additive element M as shown in FIG. 3, the residual magnetic flux density (Br) was significantly decreased. Moreover, even in the case of R-T-B system rare earth permanent magnets in which no intraphase products were observed (Comparative Examples 2 and 3), the squareness (Hk/HcJ) was improved by adding as a large amount of Zr as 0.2% by weight (refer to FIG. 5). However, a decrease in the residual magnetic flux density (Br) was still significant (refer to FIG. 3). As described above, an R-T-B system rare earth permanent magnet in which the presence of an intraphase product is observed enables to obtain a high squareness (Hk/HcJ), while inhibiting a decrease in the residual magnetic flux density (Br).

With regard to Comparative Example 3 in which an intraphase product was observed in the R₂T₁₄B phase in the stage of low R alloys, the reason why no intraphase products exist in the R-T-B system rare earth permanent magnet is assumed as follows. A Zr rich product generated in the R₂T₁₄B phase(intraphase product) in the stage of low R alloys has been grown to be extremely large. It is assumed that although this product is subjected to the hydrogen crushing process, it does not lead to volume expansion. It is therefore understood that a crack is generated on the interface between the R₂T₁₄B phase and the product during the hydrogen crushing process. When the alloys are subjected to a crushing process in this state, the product is separated from the R₂T₁₄B phase. As a result, the product is not contained in the R₂T₁₄B phase, but it exists independently from the R₂T₁₄B phase. Accordingly, it is considered that in the R-T-B system rare earth permanent magnet of Comparative Example 3, the Zr rich product exists only in the grain boundary phase even after the sintering process.

An R-T-B system rare earth permanent magnet containing 0.10% by weight of Zr in Example 1 was observed by TEM in the same manner as described above. The observation results are shown in FIGS. 6 to 8. FIG. 6 is a TEM photograph of a sample containing 0.10% by weight of Zr. FIG. 7 is a set of EDS (Energy Dispersive X-ray Fluorescence Spectrometer) profiles of a product existing in the sample and the R₂T₁₄B phase of the sample. FIG. 8 is a high resolution TEM photograph of the sample.

As shown in FIG. 6, an intraphase product with a large axis ratio can be observed in the R₂T₁₄B phase. This product has a platy or acicular form. FIG. 6 is a photograph obtained by observing the cross section of the sample, and it is therefore difficult to determine from such observation whether the form is platy or acicular. Considering the results from the observation of other samples and FIG. 8, the intraphase product has a length of several hundreds nm and a width between several nm and 15 nm. The detailed chemical composition of this intraphase product is uncertain, but from FIG. 7A, it can be confirmed that the intraphase product is at least rich in Zr. Moreover, as a result of observation of other samples, other than the intraphase product with a large axis ratio, indefinite or round shape intraphase products can also be observed, as shown in FIGS. 9 and 10. As a result of observing 20 crystal grains (R₂T₁₄B phase) of Example 1, intraphase products were observed in 6 crystal grains thereof. In contrast, in Comparative Example 2, no intraphase products were observed in any of 20 crystal grains (R₂T₁₄B phase).

The lower image of FIG. 11A shows the Zr mapping results of a sample containing 0.10% by weight of Zr of Example 1 by EPMA (Electron Probe Micro Analyzer). The upper image of FIG. 11A shows a composition image in the same scope as the Zr mapping results shown in the lower image of FIG. 11A. Moreover, the lower image of FIG. 11B shows the Zr mapping results of a sample containing 0.10% by weight of Zr of Comparative Example 2 by EPMA. The upper image of FIG. 11B shows a composition image in the same scope as the Zr mapping results shown in the lower image of FIG. 11B.

As with the results obtained by the observation by TEM, it is found from FIG. 11A that an R₂T₁₄B phase that is rich in Zr is present in the permanent magnet of Example 1, and that Zr exists also in a grain boundary phase thereof. In contrast, it is found from FIG. 11B that such a Zr rich R₂T₁₄B phase is not observed in the permanent magnet of Comparative Example 2, and that Zr exists only in a grain boundary phase thereof.

### <Embodiment Example 2>

R-T-B system rare earth permanent magnets were obtained in the same manner as in Embodiment Example 1 with the exception that samples each containing 0.10% by weight of additive element M (Zr or Ti) of the composition of the sintered body were sintered for 4 hours within the temperature range between 1,010°C and 1,090°C. The magnetic properties of the obtained permanent magnets were measured in the same manner as in Embodiment Example 1. The results are shown in FIG. 12. In addition, changes in the magnetic properties by changes in the sintering temperature are shown in FIGS. 13 to 15. Moreover, the magnetic properties at each sintering temperature plotted as a squareness (Hk/HcJ) to a residual magnetic flux density (Br) are shown in FIG. 16.

As shown in FIGS. 12 to 16, it is found that when an intraphase product is obtained by adding Zr as an additive element M, high magnetic properties are stably obtained in a wide sintering temperature range. More specifically, in Example 2 of the present invention, a residual magnetic flux density (Br) of 13.9 kG or greater, a coercive force (HcJ) of 13.0 kOe or greater, and a squareness (Hk/HcJ) of 95% or more can be obtained in the sintering temperature range between 1,030°C and 1,090°C. If Ti is added as an additive element M, the residual magnetic flux density (Br) decreases (Comparative Example 4). Moreover, when no intraphase products exist, the squareness (Hk/HcJ) is poor, and the suitable sintering temperature range is narrow (Comparative Example 5).

### <Embodiment Example 3>

Setting a roll peripheral velocity to 0.6 to 1.8 m/s, 4 types of low R alloys and 2 types of high R alloys having the compositions and thicknesses as shown in FIG. 17 were prepared by the strip casting method. Thereafter, 4 types of R-T-B system rare earth permanent magnets with the combinations as shown in FIG. 17 were obtained. In all of samples A to D, the mixing ratio between the low R alloys and the high R alloys was 90 : 10. The low R alloys and the high R alloys as shown in FIG. 17 were subj ected to hydrogen crushing in the same manner as in Embodiment Example 1. After completion of the hydrogen crushing process, 0.05% by weight of butyl oleate was added thereto. Thereafter, using a Nauta mixer, the low R alloys were mixed with the high R alloys for 30 minutes in the combinations as shown in FIG. 17. Thereafter, the mixture was subjected to the pulverizing with a jet mill to a mean particle size of 4.1 µm. The obtained fine powders were compacted in a magnetic field under the same conditions as in Embodiment Example 1, followed by sintering at 1,010°C to 1,090°C for 4 hours. Thereafter, the obtained sintered body was subjected to a two-step aging treatment consisting of treatments of 800°C × 1 hour and 550°C × 2.5 hours. The composition, the amount of oxygen, and the amount of nitrogen of each of the obtained sintered bodies are shown in FIG. 17. In addition, magnetic properties thereof are shown in FIG. 18.

As shown in FIG. 18, sample A has a residual magnetic flux density (Br) of 14.0 kG or greater, a coercive force (HcJ) of 13.0 kOe or greater, and a squareness (Hk/HcJ) of 95% or more in the sintering temperature range between 1,030°C and 1,070°C.

Samples B and C, both of which contain a lower amount of Nd than sample A, have a residual magnetic flux density (Br) of 14.0 kG or greater, a coercive force (HcJ) of 13.5 kOe or greater, and a squareness (Hk/HcJ) of 95% or more in the sintering temperature range between 1,030°C and 1,090°C.

Sample D containing a higher amount of Dy than sample Ahasaresidualmagneticflux density (Br) of 13.5 kG or greater, a coercive force (HcJ) of 15.5 kOe or greater, and a squareness (Hk/HcJ) of 95% or more in the sintering temperature range between 1,030°C and 1,070°C.

As a result of the observation of the samples sintered at 1,050°C by TEM, intraphase products were observed in all the samples.

From the above results, it can be said that when an intraphase product exists, high magnetic properties can be consistently obtained in a wide suitable sintering temperature range of 40°C or more.

### <Embodiment Example 4>

2 types of low R alloys and 2 types of high R alloys were prepared by the strip casting method. Thereafter, 2 types of R-T-B system rare earth permanent magnets with the combinations as shown in FIG. 19 were obtained. In sample E, the mixing ratio between the low R alloys and the high R alloys was 90 : 10. On the other hand, in sample F, the mixing ratio between the low R alloys and the high R alloys was 80 : 20. The low R alloys and the high R alloys as shown in FIG. 19 were subjected to hydrogen crushing in the same manner as in Embodiment Example 1. After completion of the hydrogen crushing process, 0.05% by weight of butyl oleate was added thereto. Thereafter, using a Nauta mixer, the low R alloys were mixed with the high R alloys for 30 minutes in the combinations as shown in FIG. 19. Thereafter, the mixture was subjected to the pulverizing with a jet mill to a mean particle size of 4.0 µm. The obtained fine powders were compacted in a magnetic field under the same conditions as in Embodiment Example 1. Thereafter, in the case of sample E, the compacted body was sintered at 1,070°C for 4 hours, and in the case of sample F, it was sintered at 1,020°C for 4 hours. Thereafter, the obtained sintered bodies of both samples E and F were subjected to a two-step aging treatment consisting of treatments of 800°C × 1 hour and 550°C × 2.5 hours. The composition, the amount of oxygen, and the amount of nitrogen of each of the obtained sintered bodies are shown in FIG. 19. In addition, magnetic properties thereof are shown in FIG. 20. For convenience of comparison, the magnetic properties of samples A to D prepared in Embodiment Example 3 are also shown in FIG. 20.

Although the constitutional elements were fluctuated as shown in samples A to F, a residual magnetic flux density (Br) of 13.8 kG or greater, a coercive force (HcJ) of 13.0 kOe or greater, and a squareness (Hk/HcJ) of 95% or more were obtained.

### INDUSTRIAL APPLICABILITY

As described in detail above, a Zr rich product is allowed to exist in an R₂T₁₄B phase that constitutes the main phase of an R-T-B system rare earth permanent magnet, so that the grain growth can be inhibited, while keeping a decrease in magnetic properties to a minimum. Moreover, according to the present invention, since a suitable sintering temperature range of 40°C or more can be kept, even using a large sintering furnace that is usually likely to cause unevenness in heating temperature, an R-T-B system rare earth permanent magnet consistently having high magnetic properties can be easily obtained.

## Claims

1. An R-T-B system rare earth permanent magnet, comprising a sintered body consisting of 28% to 33% by
weight of R, 0.5% to 1.5% by weight of B, 0.03% to 0.3% by weight of Al, 0.03 to 0.3% by weight of Cu, 0.05% to 0.2% by weight of Zr, 0.1% to 4% by weight of Co, and the balance substantially being Fe and unavoidable impurities
said sintered body comprising:
a main phase consisting of an R₂T₁₄B phase, wherein R represents one or more rare earth elements providing that the rare earth elements include Y, and T represents one or more transition metal elements containing Fe, or Fe and Co; and
a grain boundary phase containing a higher amount of R than said main phase,
wherein a product that is rich in Zr exists in said R₂T₁₄B phase and has a length of several hundreds nm and a width between several nm and 15 nm.

2. An R-T-B system rare earth permanent magnet according to claim 1, wherein said product has a platy or acicular form.

3. An R-T-B system rare earth permanent magnet according to claim 1, wherein the amount of oxygen contained in said sintered body is 2,000 ppm or less.

4. An R-T-B system rare earth permanent magnet according to claim 3, wherein
0.1% to 0.15% by weight of Zr is contained in said sintered body.

## Patentansprüche

1. Seltenerden-Permanentmagnet vom R-T-B-System, umfassend einen Sinterkörper, der aus 28 bis 33 Gew.% R, 0,5 bis 1,5 Gew.% B, 0,03 bis 0,3 Gew.% Al, 0,03 bis 0,3 Gew.% Cu, 0,05 bis 0,2 Gew.% Zr, 0,1 bis 4 Gew.% Co und als Rest im Wesentlichen Fe und unvermeidbaren Verunreinigungen besteht, wobei der Sinterkörper folgendes umfasst:
eine Hauptphase bestehend aus einer R₂T₁₄B-Phase, wobei R für ein oder mehrere Seltenerdelement(e) steht, mit der Bedingung, dass die Seltenerdelemente Y beinhalten, und T für ein oder mehrere Übergangsmetall-Elemente steht, die Fe oder Fe und Co beinhalten; und
eine Korngrenzenphase, die eine größere Menge an R enthält als die Hauptphase,
wobei in der genannten R₂T₁₄B-Phase ein Zr-reiches Produkt existiert, das eine Länge von einigen hundert nm und eine Breite zwischen einigen nm und 15 nm hat.

2. Seltenerden-Permanentmagnet vom R-T-B-System gemäß Anspruch 1, wobei das genannte Produkt eine flache oder nadelförmige Form hat.

3. Seltenerden-Permanentmagnet vom R-T-B-System gemäß Anspruch 1, wobei die Menge an Sauerstoff, die im genannten Sinterkörper enthalten ist, 2000 ppm oder weniger ist.

4. Seltenerden-Permanentmagnet vom R-T-B-System gemäß Anspruch 3, wobei im genannten Sinterkörper 0,1 bis 0,15 Gew.% Zr enthalten ist.

## Revendications

1. Aimant permanent à éléments en terres rares en alliage de R-T-B, comprenant un corps fritté consistant en 28% à 33% en poids de R, 0,5% à 1,5% en poids de B, 0,03% à 0,3% en poids de Al, 0,03 à 0,3% en poids de Cu, 0,05% à 0,2% en poids de Zr, 0,1 à 4% en poids de Co, et le reste étant sensiblement Fe et des impuretés inévitables.
ledit corps fritté comprenant :
une phase principale consistant en une phase R₂T₁₄B, dans laquelle R représente un ou plusieurs éléments de terres rares, à condition que les éléments de terres rares comprennent Y, et T représente un ou plusieurs éléments des métaux de transition contenant Fe, ou Fe et Co ; et
une phase de limite de grains contenant une quantité de R supérieure à ladite phase principale,
dans lequel il existe un produit qui est riche en Zr dans ladite phase R₂T₁₄B et qui a une longueur de plusieurs centaines de nm et une largeur entre plusieurs nm et 15 nm.

2. Aimant permanent à éléments en terres rares en alliage de R-T-B selon la revendication 1, dans lequel ledit produit présente une forme plate ou aciculaire.

3. Aimant permanent à éléments en terres rares en alliage de R-T-B selon la revendication 1, dans lequel la quantité d'oxygène contenue dans ledit corps fritté est de 2000 ppm ou moins.

4. Aimant permanent à éléments en terres rares en alliage de R-T-B selon la revendication 3, dans lequel
0, 1 % à 0,15% en poids de Zr est contenu dans ledit corps frittée.
